# EUROPEAN PATENT SPECIFICATION

(11) **EP 0 004 748 B1**
(45) Date of publication and mention of the grant of the patent: **14.03.1984**
(21) Application number: 79300512.5
(22) Date of filing: 29.03.1979
(51) Int. Cl.: G03G 9/08, G03G 9/10

(54) **Electrostatographic developer mixture and imaging process**
Elektrostatographisches Entwicklergemisch und Bildherstellungsverfahren
Mélange de développateur électrostatographique et procédé de formation d'images

(30) Priority: 06.04.1978 US 893915
(43) Date of publication of application: 17.10.1979
(73) Proprietor: XEROX CORPORATION, Rochester New York 14644 (US)
(72) Inventor: Volkers, Stewart W., Williamson New York 14589 (US); Webb, John L., Fairport New York 14450 (US)
(74) Representative: Goode, Ian Roy

## Description

This invention relates to an electrostatographic developer mixture, and to an electrostatographic imaging process using the developer mixture. The mixture comprises finely-divided toner particles electrostatically clinging to the surface of carrier particles.

The formation and development of images on the surface of photoconductive materials by electrostatic means is well-known. The basic electrostatographic process, as taught by C. F. Carlson in U.S. Pat. No. 2,297,691, involves placing a uniform electrostatic charge on a photoconductive insulating layer, exposing the layer to a light-and-shadow image to dissipate the charge on the areas of the layer exposed to the light and developing the resulting electrostatic latent image by depositing on the image a finely-divided electroscopic material referred to in the art as "toner".

One technique for developing an electrostatic latent image is the "magnetic brush" process as disclosed, for example, in U.S. Pat. No. 2,874,063. In this method a developer material containing toner and magnetic carrier particles is carried by a magnet. The magnetic field on the magnet causes alignment of the magnetic carriers in a brush-like configuration. This magnetic brush is engaged with an electrostatic latent image-bearing surface and the toner particles are drawn from the brush to the electrostatic image by electrostatic attraction. Many other methods such as "touchdown" development as disclosed by C. R. Mayo in U.S. Pat. No. 2,895,847 are known for applying electroscopic particles to the electrostatic latent image to be developed.

While ordinarily capable of producing good quality images, conventional developing systems suffer serious deficiencies in certain areas. In the reproduction of high contrast copies such as letters, tracings and the like, it is desirable to select the electroscopic powder and carrier materials so that their mutual. electrification is governed in most cases by the distance between their relative positions in the triboelectric series. However, when otherwise compatible electroscopic powder and carrier materials are removed from each other in the triboelectric series by too great a distance, the resulting images are very faint because the attractive forces between the carrier and toner particles compete with the attractive forces between the electrostatic latent image and the toner particles. Although the image density may be improved by increasing the toner concentration in the developer mixture, undesirably high background toner deposition as well as increased toner impaction and agglomeration is encountered when the toner concentration in the developer mixture is excessive. The initial electrostatographic plate charge may be increased to improve the density of the deposited powder image, but the plate charge would ordinarily have to be excessively high in order to attract the electroscopic powder away from the carrier particle. Excessively high electrostatographic plate charges are not only undesirable because of the high power consumption necessary to maintain the electrostatographic plate at high potentials, but also because the high potential causes the carrier particles to adhere to the electrostatographic plate surface rather than merely roll across and off the electrostatographic plate surface. Print deletion and massive carryover of carrier particles often occur when carrier particles adhere to reusable electrostatographic imaging surfaces. Massive carrier carry-over problems are particularly acute when the developer is employed in solid area coverage machines where excessive quantities of toner particles are removed from carrier particles thereby leaving many carrier particles substantially bare of toner particles. Further, adherence of carrier particles to reusable electrostatographic imaging surfaces promotes the formation of undesirable scratches on the surfaces during image transfer and surface cleaning operations. It is therefore apparent that many materials which otherwise have suitable properties for employment as developer materials are unsuitable due to their unsatisfactory electrical properties. Further, uniform triboelectric surface characteristics of many carrier surfaces are difficult to achieve with mass production techniques. Quality images are in some instances almost impossible to obtain in high speed automatic machines when carriers having non-uniform triboelectric properties are employed. The addition of large quantities of material to the original carrier material to change the triboelectric properties thereof requires a major manufacturing operation and often undesirably alters the original physical characteristics of the carrier material. Further, it is highly desirable to control the triboelectric properties of carrier surfaces to accommodate the use of desirable toner compositions while retaining the other desirable physical characteristics of the carrier. Another factor affecting the stability of the triboelectric properties of developer materials is the susceptibility of developer particles to "toner impaction". When developer particles are employed in automatic machines and recycled through many cycles, the many collisions which occur between the carrier particles and other surfaces in the machine cause the toner particles carried on the surface of the carrier particles to be welded or otherwise forced onto the carrier surfaces. The gradual accumulation of impacted toner material on the surface of the carrier causes a change in the triboelectric value of the carrier and directly contributes to the degradation of copy quality by eventual destruction of the toner carrying capacity of the carrier.

In U.S. Patent 3,942,979, there is disclosed a developer mixture comprising classified toner materials having a particle size distribution wherein less than about 30% by number of the toner particles have an average particle size diameter of less than about 5 pm, about 25% of the particles have a diameter between about 8 µm and about 12 µm and less than about 5% by number of the toner particles have an average particle diameter greater than about 20 µm. The high surface area carrier materials have a specific surface of at least about 150 cm²/gram. It is also indicated therein that for cascade and magnetic brush development, the carrier particles generally have an average diameter between about 30 µm and 1000 µm, and between about 30 and about 250 µm respectively. In the case of magnetic brush development, the preferred carrier has a majority of the carrier particles in the range 74 to 105 µm.

In DE-A-2 261 593 there is disclosed a developer mixture comprising toner particles and carrier particles, in which the carrier particles comprise a mixture of small and large particles. The toner particles are in the size range 5 to 20 µm, the small carrier particles from 1 to 25 µm and the large carrier particles from 15 to 200 µm. In a typical mixture, the toner particles range from 8 to 15 µm, with a main particle size of 10-11 pm. Most of the large carrier particles are from 30 to 80 µm in size with the most numerous size being 50-52 µm, and most of the small carrier particles are from 5 to 16 µm in size with the most numerous particle size being 15-16 µm.

Present commercial magnetic brush development systems generally employ carrier particles that are approximately 100 µm in diameter. Toner particles employed with these carrier particles typically have a distribution of particle sizes that vary from 1 to 30 µm. Experience with the aforementioned developer materials reveals degradation of copy quafity as reflected by blurred and mottled prints having poor edge acuity and resolution.

Thus, there is a continuing need for better developer materials for developing electrostatic latent images.

The invention as claimed is intended to provide developer materials which overcome the above noted deficiencies. This is achieved by the use of a developer mixture which is characterised in that the toner particles are of a size between a lower size limit of 3 µm and an upper size limit of 10. µm, particles of sizes smaller than the lower size limit and larger than the upper size limit having been removed, and in that the carrier particles have a size between 10 and 40 µm.

Good results are obtained when the toner materials have a particle size in the range of between 3 µm and 10 µm and the carrier materials have a mean particle size in the range of between 10 µm and 40 µm.

The invention offers the advantages of developer materials having more stable electrostatographic properties, improved triboelectric properties and a longer useful life. These developer materials are less susceptible to toner impaction, they are more resistant to film formation, i.e. the formation of a thin film of toner material, on electrostatographic recording surfaces, and enable the attainment of copied images having greatly improved quality.

Various ways of carrying out the invention will now be described.

It has now been found that the removal from toner materials of toner particles which are below about 3 ₁₁m will provide a developer mixture having improved carrier life, background deposits are minimized, and photoreceptor cleaning is greatly facilitated. More particularly, toner particles having a diameter below 3 µm usually encompass free colorant such as carbon black, and unpigmented platelets which are undesirable since they inhibit proper triboelectric charging and reduce the active carrier surface area resulting in high background deposition of such particles.

By considering the particle size of toner particles relative to copy quality, a particle size range of 3 to 10 µm with a mean particle size of about 8 pm has been found to provide maximum copy quality. Apparently, toner particles having a diameter below 3 microns are triboelectrically charged too highly and they tend to not be developed as easily as the larger particles and also prevent the larger particles from being charged high enough. These lower charged larger particles are difficult to control in a developer mixture and will usually undesirably develop onto the background areas of an electrostatic latent image.

It has also been found that the removal from toner materials of toner particles having a diameter larger than 10 µm will provide improved copy quality since such particles have been found to produce observable blur in biased transfer roll systems.

It has also been found that conventional 100 µm size carrier particles are very quickly impacted with toner particles thus reducing the useful life of such developer mixtures. Thus, in accordance with this invention, by employing toner particles having a diameter between 3 and 10 µm with carrier particles having a diameter of between 10 and 40 µm, this carrier size range increases the surface area of the carrier material to accommodate the toner material as described above and the carrier particles have lower energies available for causing damage on impact. The net result of the developer mixtures of this invention is the provision of prints produced by the electrostatographic process wherein the printed image now has improved edge acuity, high resolution, and sharp, crisp characters. Where an occasional toner particle deposits in background areas, due to the smaller size of the toner particles employed, the background deposit is not perceivable by the naked eye. Likewise, due to the smaller size of the carrier particles employed in the developer mixtures of this invention, it is now possible for the carrier particles to carry sufficient toner particles to enable development of large solid areas without employing excessively high toner concentrations which previously led to unacceptably high image background deposits.

Pursuant to this invention, the enhanced surface/volume ratio of the developer mass provides increased toner carrying capacity and consequently improved toner concentration latitude. In addition, the developer materials of this invention provide improved insulation between adjacent carrier beads when the carrier particles are made of a conductive metal and the carrier particles do not contain a coating of an insulating material. This is due to the increased population of toner particles between contacting carrier particles which improves the resistance to shorting between conductive carrier particles and the photoreceptor. As indicated, the carrier material should preferably be conductive to realize the virtual electrode effect for maximum development and to prevent build-up of net electrical charge. The combination of developer materials of this invention has been found to provide prints of outstanding high quality which are indistinguishable from offset prints.

It has further been found that the developer compositions of this invention provide developed images having a more uniform and lower pile height than achieved with conventional electrostatographic developer compositions. For example, when employing conventional developer compositions in a high speed electrostatographic copying/duplicating machine, such as the Xerox 9200, the developed, unfused image toner pile height is between about 45 and 55 pm. 'Xerox' and '9200' are Registered Trade Marks. However, when employing the novel developer compositions of this invention in the same machine, the developed, unfused image toner pile height is only about 18 pm. In both instances, the image density is about 1.3 but the lower toner pile height obtained with the compositions of this invention is due to their greater covering power; that is, a greater number of toner particles are packed closer together, absorbing more reflected light, and therefore the perceived image density is the same in both cases yet the toner pile height is much less with these new developer materials. This finding is significant since there has conventionally been a substantial disparity in toner pile height between developed, unfused solid image areas and developed, unfused line image areas. However, with the developer compositions of this invention, the toner pile height of developed, unfused solid image areas and that of developed, unfused line image areas is substantially the same. Thus, with uniform toner pile heights in both the solid image areas and the line image areas, it is now possible to obtain a transferred and fused image having a more uniform output density and a greatly improved physical appearance. This is due to greatly improved toner image transfer to a permanent substrate such as paper since, in conventional transfer systems, toner particle size and toner pile height affect transfer efficiency. That is, excessively small toner particles were previously left behind on the photoreceptor during transfer resulting in wasted toner, a non-uniform transferred image was obtained, and photoreceptor cleaning problems were aggravated. However, with efficient transfer of developed, unfused solid and line image areas having uniform and lower toner pile heights, fusing of the toner material is more efficient, more uniform, and requires substantially less energy. Also, since less fusing energy is required, copy paper degradation problems such as curling, reduced moisture content, resistivity, and paper transport problems are minimized.

Any suitable particle classification method may be employed to obtain the toner materials of this invention. Typical particle classification methods include air classification, screening, cyclone separation, elutriation, centrifugal separation, and combinations thereof. The preferred method of obtaining the toner materials of this invention is by centrifugal air classification. In this method, air or some other gas flows inwards in a spiral path through a flat, cylindrical chamber. Particles contained in the air flow are exposed to two antagonistic forces, viz., to the inwardly directed tractive force of the air, and to the outwardly directed centrifugal force of the particle. For a definite size of particles, that is, the "cut size", both forces are in equilibrium. Larger (heavier) particles are dominated by the mass-dependent centrifugal force and the smaller (lighter) particles by the frictional force proportional to the particle diameter. Consequently, the larger or heavier particles fly outwards as coarse fraction, while the smaller or lighter ones are carried inwards by the air as fine fraction. The "cut size" usually depends upon the gradient of the spiral, the peripheral component, and the absolute dimension of the classifying chamber. Adjustment of the cut size may be effected through variation of the two factors first mentioned, while the range of the cut size may be determined by the respective dimension of the classifying chamber. Satisfactory centrifugal air classification results may be obtained when employing an apparatus such as the Mikroplex Spiral Air Classifier Type 132MP model available from the Alpine American Corporation, Natick, Massachusetts, or an Acucut Model B18 unit available from the Donaldson Company, Inc., Tulsa, Oklahoma.

Any suitable particle classification method may be employed to obtain the carrier materials of this invention. Typical particle classification methods include air classification, screening, cyclone separation, elutriation, centrifugal separation and combinations thereof. The preferred method of obtaining the carrier materials of this invention is by screening or sieving.

Any suitable vinyl resin having a melting point of at least about 110°F may be employed in the toner compositions. The vinyl resin may be a homopolymer or a copolymer of two or more vinyl monomers. Typical monomeric units which may be employed to form vinyl polymers include: styrene, p-chloro-styrene, vinyl naphthalene; ethylenically unsaturated monoolefins such as ethylene, propylene, butylene, isobutylene and the like; vinyl halides such as vinyl chloride, vinyl bromide, vinyl fluoride; vinyl esters such as vinyl acetate, vinyl propionate, vinyl benzoate, vinyl butyrate and the like; esters of alphamethylene aliphatic monocarboxylic acids such as methyl acrylate, ethyl acrylate, n-butylacrylate, isobutyl acrylate, dodecyl acrylate, n-octyl acrylate, 2-chloroethyl acrylate, phenyl acrylate, methyl-alpha- chloroacrylate, methyl methacrylate, ethyl methacrylate, butyl methacrylate and the like; acrylonitrile, methacrylonitrile, acrylamide, vinyl ethers such as vinyl methyl ether, vinyl isobutyl ether, vinyl ethyl ether, and the like; vinyl ketones such as vinyl methyl ketone, vinyl hexyl ketone, methyl isopropenyl ketone and the like; vinylidene halides such as vinylidene chloride, vinylidene chlorofluoride and the like; and N-vinyl compounds such as N-vinyl pyrrole, N-vinyl carbazole, N-vinyl indole, N-vinyl pyrrolidine and the like, and mixtures thereof. Generally, suitable vinyl resins employed in the toner have a weight average molecular weight between about 3,000 to about 500,000.

Toner resins containing relatively high percentages of a styrene resin are preferred. The presence of a styrene resin is preferred because a greater degree of image definition is generally achieved upon latent image development. Further, denser images are obtained when at least about 25 percent by weight, based on the total weight of resin in the toner, of a styrene resin is present in the toner. The styrene resin may be a homopolymer of styrene or styrene homologues or copolymers of styrene with other monomeric groups containing a single methylene group attached to a carbon atom by a double bond. Thus, typical monomeric materials which may be copolymerized with styrene by addition polymerization include: P-chlorostyrene, vinyl naphthalene, ethylenically unsaturated monoolefins such as ethylene, propylene, butylene, isobutylene and the like; vinyl esters such as vinyl chloride, vinyl bromide, vinyl fluoride, vinyl acetate, vinyl pro- ^{p}ionate, vinvl benzoate. vinvl butvrate and the like; esters of alpha-methylene aliphatic monocarboxylic acids such as methyl acrylate, ethyl acrylate, n-butylacrylate, isobutyl acrylate, dodecyl acrylate, n-octyl acrylate, 2-chloroethyl acrylate, phenyl acrylate, methyl-alpha- chloroacrylate, methyl methacrylate, ethyl methacrylate, butyl methacrylate and the like; acrylonitrile, methacrylonitrile, acrylamide, vinyl ethers such as vinyl methyl ether, vinyl isobutyl ether, vinyl ethyl ether, and the like; vinyl ketones such as vinyl methyl ketone, vinyl hexyl ketone, methyl isopropenyl ketone and the like; vinylidene halides such as vinylidene chloride, vinylidene chlorofluoride and the like; and N-vinyl compounds such as N-vinyl pyrrole, N-vinyl carbazole, N-vinyl indole, N-vinyl pyrrolidine and the like; and mixtures thereof. The styrene resins may also be formed by the polymerization of mixtures of two or more of these unsaturated monomeric materials with a styrene monomer.

The vinyl resins, including styrene type resins, may also be blended with one or more other resins if desired. When the vinyl resin is blended with another resin, the added resin is preferably another vinyl resin because the resulting blend is characterized by especially good triboelectric stability and uniform resistance against physical degradation. The vinyl resins employed for blending with the styrene type or other vinyl resin may be prepared by the addition polymerization of any suitable vinyl monomer such as the vinyl monomers described above. Other resins may also be blended with the vinyl resins of this invention. Typical non-vinyl resins include: rosin modified phenol formaldehyde, resins, oil modified epoxy resins, polyurethane resins, cellulosic resins, polyether resins and mixtures thereof. When the resin component of the toner contains styrene copolymerized with another unsaturated monomer or a blend of polystyrene and another resin, a styrene component of at least about 25 percent by weight based on the total weight of the resin present in the toner is preferred because denser images are obtained and a greater degree of image definition is achieved with a given quantity of toner material.

It is to be understood that the specific formulae given for the units contained in the resins of the toner materials represent the vast majority of the units present, but do not exclude the presence of monomeric units or reactants other than those which have been shown. For example, some commercial materials contain trace amounts of homologues or unreacted or partially reacted monomers. Any minor amount of such substituents may be present in the materials of this invention.

Any suitable pigment or dye may be employed as the colorant for the toner particles. Toner colorants are well-known and include, for example, carbon black, nigrosine dye, aniline blue, Calco Oil Blue, chrome yellow, ultramarine blue duPont Oil Red, Quinoline Yellow, methylene blue chloride, phthalocyanine blue, Malachite Green Oxalate, lamp black, Rose Bengal and mixtures thereof. The pigment or dye should be present in the toner in a quantity sufficient to render it highly coloured so that it will form a clearly visible image on a recording member. Thus, for example, where conventional electrostatographic copies of typed documents are desired, the toner may comprise a black pigment such as carbon black, for example, furnace black or channel black, or a black dye such as Amaplast Black dye, available from the National Aniline Products, Inc. Generally, the pigment is employed in an amount from about 1 percent to about 20 percent by weight based on the total weight of the coloured toner. If the toner colorant employed is a dye, substantially smaller quantities of colorant may be used. However, since a number of the above pigments used in electrostatographic toner compositions may affect both the glass transition and fusion temperatures of the toner compositions of this invention, their concentration preferably should be less than about 10 percent by weight of the colored toner. Representative patents in which toner and developer materials are disclosed include U.S. Patent 2,788,288, U.S. Patent 3,079,342, U.S. Reissue Patent 25,136, U.S. Patent 3,577,345, U.S. Patent 3,653,893, U.S. Patent 3,590,000, U.S. Patent 3,655,374, U.S. Patent 3,720,617, and U.S. Patent 3,819,367. Especially preferred for use in the present invention are those compositions disclosed in U.S. Reissue Patent 25,136 and U.S. Patent 3,079,342 containing a copolymer of styrene and alkyl methacrylate; the compositions disclosed in U.S. Patent 3,590,000 comprising a solid, stable hydrophilic metal salt of a fatty acid such as zinc stearate, and a polymeric esterification product of a dicarboxylic acid and a diol comprising a diphenol; and the compositions disclosed in U.S. Patent 3,819,367 containing a minor proportion of submicroscopic silicon dioxide additive particles.

The toner compositions may be prepared by a well-known toner mixing and comminution technique. For example, the ingredients may be thoroughly mixed by blending, mixing and milling the components and thereafter micro- pulverizing the resulting mixture. Another well-known technique for forming toner particles is to spray-dry a ball-milled toner composition comprising a colorant, a resin, and a solvent.

Any suitable coated or uncoated electrostatographic carrier bead material may be employed as the carrier material of this invention. Typical carriers include sodium chloride, ammonium chloride, aluminium potassium chloride. Rochelle salt, sodium nitrate, aluminium nitrate, potassium chlorate, granular zircon, granular silicon, methyl methacrylate, glass and silicon dioxide. Typical magnetic brush development process carriers include nickel, steel iron, ferrites, and the like, and are preferred in the compositions of this invention. The carriers may be employed with or without a coating. Many of the foregoing and other typical carriers are described by L. E. Walkup, et al in U.S. Pat. No. 2,638,416 and E. N. Wise in U.S. Pat. No. 2,618,552. Additionally, it is preferred that the carrier materials have semiconductive to conductive properties. Where desired, the carrier materials of this invention may be coated with any suitable insulating material. Typical electrostatographic carrier particle coating materials include vinyl chloride-vinyl acetate copolymers, styrene- acrylate-organosilicon terpolymers, natural resins such as caoutchouc, colophony, copal, dammar, jalap, storax; thermoplastic resins including the polyolefins such as polyethylene, polypropylene, chlorinated polyethylene, and chlorosulfonated polyethylene; polyvinyls and polyvinylidenes such as polystyrene, poly- methylstyrene, polymethyl methacrylate, polyacrylonitrile, polyvinyl acetate, polyvinyl alcohol, polyvinyl butyral, polyvinyl chloride, polyvinyl carbazole, polyvinyl ethers, and polyvinyl ketones; fluorocarbons such as polytetrafluoroethylene, polyvinyl fluoride, polyvinylidene fluoride; and polychlorotrifluoroethylene; polyamides such as polycaprolactam and polyhexamethylene adipamide; polyesters such as polyethylene terephthalate; polyurethanes; polysulfides, polycarbonates, thermosetting resins including phenolic resins such as phenolformaldehyde, phenol-furfural and resorcinol formaldehyde; amino resins such as ureaformaldehyde and melamine-formaldehyde; polyester resins; epoxy resins; and the like. Many of the foregoing and other typical carrier coating materials are described by L. E. Walkup in U.S. Pat. No. 2,618,551; B. B. Jacknow, et al. in U.S. Pat. No. 3,526,433; and R. J. Hagenbach, et al. in U.S. Pat. Nos. 3,533,835 and 3,658,500.

When the carrier materials of this invention are coated, any suitable electrostatographic carrier coating thickness may be employed. However, a carrier coating having a thickness of at least sufficient to form a thin film on the carrier particle is preferred because the carrier coating will then possess sufficient thickness to resist abrasion and prevent pinholes which adversely affect the triboelectric properties of the coated carrier particles. Generally, for cascade and magnetic brush development, the carrier coating may comprise from about 0.1 percent to about 10.0 percent by weight based on the weight of the coated carrier particles. Preferably, the carrier coating should comprise from about 0.3 percent to about 1.5 percent by weight based on the weight of the coated carrier particles because maximum durability, toner impaction resistance, and copy quality are achieved. To achieve further variation in the properties of the coated composite carrier particles, well-known additives such as plasticizers, reactive and non-reactive polymers, dyes, pigments, wetting agents and mixtures thereof may be mixed with the coating materials and the coating may be continuous or discontinuous.

When the carrier materials of this invention are coated, the carrier coating composition may be applied to the carrier cores by any conventional method such as spraying, dipping, fluidized bed coating, tumbling, brushing, and the like. The coating compositions may be applied as a powder, a dispersion, solution, emulsion or hot melt. When applied as a solution, any suitable solvent may be employed. Solvents having relatively low boiling points are preferred because less energy and time is required to remove the solvent subsequent to application of the coating to the carrier cores. If desired, the coating may comprise resin monomers which are polymerized in situ on the surface of the cores or plastisols gelled in situ to a non-flowable state on the surface of the cores. Surprisingly, increased carrier active area increases the net toner material triboelectric charge level for a given toner concentration by weight in a developer mixture. Therefore, where it is preferred to operate an electrostatographic development system at a minimum toner concentration as to provide solid area coverage and at a toner concentration high enough to minimize toner deposits in background areas of a developed electrostatic latent image resulting from toner particles having a low or weak triboelectric charge, these objectives may be attained by employing the developer materials of this invention. In accordance with this invention, the aforementioned objectives are attained by operating at an increased toner concentration yet providing lower background deposits and enabling longer developer life.

Any suitable organic or inorganic photoconductive material may be employed as the recording surface with the developer materials of this invention. Typical inorganic photoconductor materials include: sulfur, selenium, zinc sulfide, zinc oxide, zinc cadmium sulfide, zinc magnesium oxide, cadmium selenide, zinc silicate, calcium strontium sulfide, cadmium sulfide, mercuric iodide, mercuric oxide, mercuric sulfide, indium trisulfide, gallium selenide, arsenic disulfide, arsenic trisulfide, arsenic triselenide, antimony trisulfide, cadmium sulfoselenide and mixtures thereof. Typical organic photoconductors include: quinacridone pigments, phthalocyanine pigments, triphenylamine, 2,4 - bis(4,4' - diethylamino- phenol) - 1, 3,4 - oxadiazol, N - isopropyl- carbazole, triphenylpyrrole, 4,5 - diphenyl- imidazolidinone, 4,5 - diphenyl - imidazolidine- thione, 4,5 - bis(4' - amino - phenyl) - imidazoli- dinoile, 1,5 - dicyanonaphthalene, 1,4 - dicyanonaphthalene, aminophthalodinitrile, nitrophthalodinitrile, 1,2,5,6 - tetraazacyclo- octatetracene - 2,4,6,8), 2 - mercaptobenzothiazole - 2 - phenyl - 4 - bisphenylideneoxa- zolone, 6 - hydroxy - 2, 3 - di(p - methoxyphenyl) - benzofurane, 4 - dimethylaminobenzylidene - benzhydrazide, 3 - benzylideneaminocarbazole, polyvinyl carbazole, (2 - nitrobenzylidene) - p - bromoanile, 2,4 - diphenylquinazoline, 1,2,4 - triazine, 5 - diphenyl - 3 - methyl - pyrazoline, 2 - (4' - dimethylaminophenyl) - benzoxazole, 3 - aminocarbazole, and mixtures thereof. Representative patents in which photoconductive materials are disclosed include U.S. Pat. No. 2,803,542 to Ullrich, U.S. Pat. No. 2,970,906 to Bixby, U.S. Pat. No. 3,121,006 to Middleton, and U.S. Pat. No. 3,151,982 to Corrsin.

The following -examples further define, describe and compare methods of preparing the developer materials of the present invention and of utilizing them to develop electrostatic latent images. Parts and percentages are by weight unless otherwise indicated.

### Example I

A control developer mixture is prepared by mixing a toner composition comprising a mixture of 90 parts by weight of a copolymer of 58.0 percent by weight of styrene and 42.0 percent by weight of n-butyl methacrylate, and 10 parts by weight of a furnace carbon black with carrier particles. The toner particles were determined to have a particle size of between 8 and 30,um. The carrier particles comprised 100 µm nickel-zinc ferrite coated with 0.6 percent by weight, based on the weight of the core material, of a carrier coating composition comprising styrene, a methacrylate ester, and an organosilicon compound as disclosed in U.S. Pat. No. 3,526,533. The coated ferrite carrier material was determined to have a specific surface area of about 151 cm²/gram.

About 1 part by weight of the toner particles was mixed with about 100 parts by weight of the carrier particles to form the developer mixture. Copies of a standard test pattern were made with the developer mixture in an electrostatographic copying machine employing a magnetic brush development system. It was found that the developer mixture failed after about 300,000 copies. Developer failure was experienced in the form of high background, i.e., exceeding the specified 0.01 background density level at 1.0 solid area density. A high level of photoreceptor filming, i.e. disposition of a thin film of toner material on the photoreceptor, was observed as print-out on the copies which occurred at a frequency of about every 60,000 intervals. The rate of toner impaction was found to be about 8 mg/g. The copies produced were found to have blurred images, with poor edge acuity. Grey scale and half-tone reproduction quality was poor. Copy resolution was less than 7 line pairs per millimetre and the presence of hollow characters was substantial.

### Example II

A developer mixture was prepared by mixing about 3 parts of the toner material employed in Example I with about 100 parts of carrier material except that the toner particles were selected to have a particle size of between 3 and 10 µm. The carrier particles were selected to comprise 35 micron nickel powder. The nickel powder was determined to have a specific surface area of about 450 cm²/gram.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was insignificant and not measurable using existing techniques.

The copies produced contained images free of blur and edge acuity was excellent. Grey scale and half-tone reproduction quality was excellent. Copy resolution was about 10 line pairs per millimetre and no hollow characters were evident.

### Example III

A developer mixture was prepared by mixing about 3 parts by weight of a toner composition comprising a mixture of 88.5 parts by weight of a polymeric esterification product of a dicarboxylic acid and a diol comprising a diphenol, and 11.5 parts by weight of a carbon black as disclosed in U.S. Patent 3,590,000 with about 100 parts by weight of carrier particles. The toner particles were selected to have a particle size of between 3 and 10 ,um. The carrier particles comprised 35 ,um nickel powder. By calculation, the nickel powder was determined to have a specific surface area of about 450 cm²/gram.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was insignificant and not measurable using existing techniques.

The copies produced contained images free of blur and edge acuity was excellent. Grey scale and half-tone reproduction quality was excellent. Copy resolution was about 10 line pairs per millimetre and no hollow characters were evident.

### Example IV

A developer mixture was prepared by mixing about 3 parts of the toner material employed in Example III with about 100 parts of the carrier material employed in Example III except that 0.65 parts by weight of submicroscopic silicon dioxide particles (Aerosil (Registered Trade Mark) R-972) based on the weight of the toner particles as described in U.S. Patent 3,819,367 was added to the developer mixture.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was excellent and not measurable using existing techniques.

The copies produced contained images free of blur and edge acuity was excellent. Grey scale and half-tone reproduction quality was excellent. Copy resolution was about 10 line pairs per millimetre and no hollow characters were evident.

### Example V

A developer mixture was prepared as in Example IV except that 0.35 parts by weight of zinc stearate based on the weight of the toner particles as described in U.S. Patent 3,590,000 was added to the developer mixture.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was insignificant and was not measurable using existing techniques.

The copies produced contained images free of blur and edge acuity was excellent. Grey scale and half-tone reproduction quality was excellent. Copy resolution was about 10 line pairs per millimetre and no hollow characters were evident.

### Example VI

A developer mixture was prepared by mixing about 3 parts by weight of a toner composition comprising a mixture of 80 parts by weight of styrene, 20 parts by weight of isobutyl methacrylate, and 10 parts by weight of a carbon black with about 100 parts by weight of carrier particles. The toner particles were determined to have a particle size of between 3 and 1Oµm. The carrier particles comprised 35 µm nickel powder.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was insignificant and not measurable using existing techniques.

The copies produced contained images free of blur and edge acuity was excellent. Grey scale and half-tone reproduction quality was excellent. Copy resolution was about 10 line pairs per millimetre and no hollow characters were evident.

### Example VII

A developer mixture was prepared by mixing about 3 parts by weight of a toner composition comprising a mixture of 80 parts by weight of styrene, 20 parts by weight of isobutyl methacrylate, 15 parts by weight of diphenyl isophthalate, and 10 parts by weight of a carbon black with about 100 parts by weight of carrier particles. The toner particles were determined to have a particle size of between 3 and 10 pm. The carrier particles comprised 35 ,um nickel powder.

The developer mixture was used to develop an electrostatic latent image under substantially the same conditions as in Example I. It was found that the developer mixture performed satisfactorily up to about 300,000 copies after which the test was suspended. No photoreceptor filming was observed as print-out on the copies. The rate of toner impaction was insignificant and not measurable using existing techniques.

The copies produced contained images free of blur and edge acuity was excellent. Grey scale and half-tone reproduction quality was excellent. Copy resolution was about 10 line pairs per millimetre and no hollow characters were evident.

Thus, the developer materials of this invention are characterized as providing substantially improved copy quality in the development of electrostatic latent images. It is believed that developed image resolution is improved due to the toner particle size range. The improved edge acuity is believed to result from less edge raking by the smaller carrier particles in the present developer mixtures. The reduced mottle appearance and absence of hollow characters of copied images obtained appears to result from more uniform latent image development and image transfer due to more uniform triboelectric charge of the developer materials. Improved grey scale and half-tone reproduction obtained with the developer materials of this invention appears to be due to the high developability of these smaller toner particles and the virtual electrode effect at the photoreceptor surface of the smaller conductive carrier particles. In addition, developer materials of this invention are further characterized as resulting in improved machine performance with longer systems life, that is, these developer materials provide substantially improved triboelectric charging properties of the developer mixtures'for substantially longer periods of time thereby increasing the developer life of the developer mixtures and decreasing the time intervals between replacement of the developer materials. Further still, the developer materials of this invention may be characterized as providing dense images and are particularly useful in magnetic brush development systems. Thus, by providing the developer materials of this invention, substantial improvements in systems life and copy quality result upon the use of developer materials having the specified physical characteristics.

In addition, the developer materials of this invention may be further characterized as experiencing substantially reduced impaction rates resulting in more stable triboelectric charging properties of the developer mixtures for substantially longer periods of time thereby increasing the developer life of the developer mixtures and decreasing the time intervals between replacement of the developer materials.

## Claims

1. An electrostatographic developer mixture comprising finely-divided toner particles electrostatically clinging to the surface of carrier particles, characterised in that the toner particles are of a size between a lower size limit of 3 pm and an upper size limit of 10 am, particles of sizes smaller than the lower size limit and larger than the upper size limit having been removed, and in that the carrier particles have a mean size between 10 and 40 ₗim.

2. An electrostatographic developer mixture in accordance with Claim 1, wherein said carrier particles comprise a conductive metal such as nickel, steel, iron, or ferrite.

3. An electrostatographic developer mixture in accordance with Claim 1 or Claim 2, wherein said carrier particles comprise a core having a coating of an insulating material.

4. An electrostatographic developer mixture in accordance with Claim 3, wherein said insulating material comprises from 0.1% to 10.0% by weight based on the weight of said carrier particles.

5. An electrostatographic developer mixture in accordance with any one of Claims 1 to 4, wherein said toner particles comprise a mixture of 90 parts by weight of a copolymer of 58.0% by weight of styrene, 42.0% by weight of n-butyl-methacrylate, and 10 parts by weight of a furnace carbon black.

6. An electrostatographic developer mixture in accordance with any one of Claims 1 to 4, wherein said toner particles comprise a mixture of 88.5 parts by weight of a polymeric esterification product of a dicarboxylic acid and a diol comprising a diphenol and 11.5 parts by weight of carbon black.

7. An electrostatographic developer mixture in accordance with Claim 6 including 0.65 parts by weight based on the weight of said toner particles of submicroscopic silicon dioxide particles.

8. An electrostatographic developer mixture in accordance with Claim 7 including 0.35 parts by weight based on the weight of said toner particles of zinc stearate.

9. An electrostatographic developer mixture in accordance with any one of Claims 1 to 4, wherein said toner particles comprise a mixture of 80 parts by weight of styrene, 20 parts by weight of isobutyl methacrylate, 15 parts by weight of diphenyl isophthalate, and 10 parts by weight of carbon black.

10. An electrostatographic imaging process comprising the steps of providing an electrostatographic imaging member having a recording surface, forming an electrostatic latent image on said recording surface, and contacting said electrostatic latent image with a developer mixture comprising finely-divided toner particles electrostatically clinging to the surface of carrier particles, characterised in that the developer mixture comprises a mixture in accordance with any one of Claims 1 to 9.

## Patentansprüche

1. Elektrostatographische Entwicklermischung, umfassend feinverteilte Tonerteilchen, die elektrostatisch an der Oberfläche von Trägerteilchen anhaften, dadurch, gekennzeichnet, daß die Tonerteilchen eine Größe zwischen einer unteren Größengrenze von 3,um und einer oberen Größengrenze von 10 µm besitzen, wobei Teilchen mit Größen unterhalb der unteren Größengrenze und oberhalb der ober Größengrenze entfernt worden sind, und daß die Trägerteilchen eine mittlere Teilchengröße zwischen 10 und 40 µm besitzen.

2. Elektrostatographische Entwicklermischung nach Anspruch 1, dadurch gekennzeichnet, daß die Trägerteilchen ein leitendes Metall, wie etwa Nickel, Stahl, Eisen oder Ferrit, aufweisen.

3. Elektrostatographische Entwicklermischung nach Anspruch 1 oder 2, dadurch gekennzeichnet, daß die Trägerteilchen einen Kern mit einer Beschichtung aus einem Isolationsmaterial aufweisen.

4. Elektrostatographische Entwicklermischung nach Anspruch 3, dadurch gekennzeichnet, daß das Isolationsmaterial 0,1 bis 10,0 Gew.-%, bezogen auf das Gewicht der Trägerteilchen, ausmacht.

5. Elektrostatographische Entwicklermischung nach mindestens einem der Ansprüche 1 bis 4, dadurch gekennzeichnet, daß die Tonerteilchen eine Mischung aus 90 Gewichtsteilen eines Copolymers aus 58,0 Gew.-% Styrol, 42,0 Gew.-% n-Butylmethacrylat, und 10 Gewichtsteileneines Ofenruss umfassen.

6. Elektrostatographische Entwicklermischung nach mindestens einem der Ansprüche 1 bis 4, dadurch gekennzeichnet, daß die Tonerteilchen eine Mischung aus 88,5 Gewichtsteilen eines polymeren Veresterungsproduktes aus einer Dicarbonsäure und einem ein Diphenol umfassenden Diol und 11,5 Gewichtsteilen Ruß umfassen.

7. Elektrostatographische Entwicklermischung nach Anspruch 6, dadurch gekennzeichnet, daß sie 0.65 Gewichtsteile, bezogen auf das Gewicht der Tonerteilchen, submikroskopische Siliciumdioxid-Teilchen beinhaltet.

8. Elektrostatographische Entwicklermischung nach Anspruch 7, dadurch gekennzeichnet, daß sie 0,35 Gewichtsteile, bezogen auf das Gewicht der Tonerteilchen, Zinksteatrat beinhaltet.

9. Elektrostatographische Entwicklermischung nach mindestens einem der Ansprüche 1 bis 4, dadurch gekennzeichnet, daß die Tonerteilchen eine Mischung aus 80 Gewichtsteilen Styrol, 20 Gewichtsteilen Isobutylmethacrylate, 15 Gewichtsteilen Diphenylisophtalat und 10 Gewichtsteilen Ruß umfassen.

10. Elektrostatographisches Abbildungsverfahren, umfassend die Stufen des Vorsehens eines elektrostatographischen Abbildungselements mit einer Aufzeichnungsfläche, Bilden eines elektrostatischen latenten Bildes auf der Aufzeichnungsfläche und Kontaktieren des elektrostatischen latenten Bildes mit einer Entwicklermischung, umfassend feinverteilte Tonerteilchen, die elektrostatisch an der Oberfläche von Trägerteilchen anhaften, dadurch gekennzeichnet, daß die Entwicklermischung eine Mischung nach mindestens einem der Ansprüche 1 bis 9 umfaßt.

## Revendications

1. Mélange pour développement électro- statographique, comprenant des particules de toner, sous forme finement divisée, adhérant électrostatiquement sur la surface de particules porteuses, caractérisé en ce que les particules de toner sont de dimensions comprises entre une limite inférieure de 3 µm et une limite supérieure de 10 p,m, après enlèvement des particules de dimensions inférieures à la limite inférieure et des particules de dimensions supérieures à la limite supérieure, et en ce que les particules porteuses sont de dimensions moyennes comprises entre 10 et 40 µm.

2. Mélange pour développement électro- statographique, selon la revendication 1, dans lequel lesdites particules porteuses comprennent un métal conducteur, tel que le nickel, l'acier ou le fer, ou de la ferrite.

3. Mélange pour développement électro- statographique, selon la revendication 1 ou la revendication 2, dans lequel lesdites particules porteuses comprennent un noyau muni d'un revêtement en une matière isolante.

4. Mélange pour développement électro- statographique, selon la revendication 3, dans lequel ladite matière isolante constitue 0,1 à 10,0%, en poids, de la massé desdites particules porteuses.

5. Mélange pour développement électro- statographique, selon l'une quelconque des revendications 1 à 4, dans lequel lesdites particules de toner comprennent un mélange de 90 parties en poids d'un copolymère à 58,0% en poids de styrène et 42,0% en poids de n-butyl-méthacrylate et de 10 parties en poids de noir de fumée.

6. Mélange pour développement électrostatique, selon l'une quelconque des revendications 1 à 4, dans lequel lesdites particules de toner comprennent un mélange de 88,5 parties en poids d'un polymère produit par estérification d'un acide dicarboxylique et d'un diol comprenant un diphénol et de 11,5 parties en poids de noir de fumée.

7. Mélange pour développement électrostatique, selon la revendication 6, comprenant 0,65 parties en poids, par rapport au poids des particules de toner, de particules de bioxyde de silicium submicroscopiques.

8. Mélange pour développement électrostatique, selon la revendication 7, comprenant 0,35 parties en poids, par rapport au poids des particules de toner, de stéarate de zinc.

9.. Mélange pour développement électrostatique, selon l'une quelconque des revendications 1 à 4, dans lequel lesdites particules de toner comprennent un mélange de 80 parties en poids de styrène, 20 parties en poids de méthacrylate, d'isobutyle, 15 parties en poids d'isophtalate de diphényle et 10 parties en poids de noir de fumée.

10. Procédé de formation d'image électrostatique, comprenant les opérations consistant à fournir un organe de formation d'image électrostatique ayant une surface d'enregistrement, à former une image latent électrostatique sur cette surface et à mettre en contact cette image latente électrostatique avec un mélange pour développement comprenant des particules de toner, sous forme finement divisée, adhérant électrostatiquement sur la surface de particules porteuses, caractérisé en ce que le mélange pour développement comprend un mélange selon l'une quelconque des revendications 1 à 9.
